# EUROPEAN PATENT SPECIFICATION

(11) **EP 0 650 184 B1**
(45) Date of publication and mention of the grant of the patent: **05.06.2002**
(21) Application number: 93914987.8
(22) Date of filing: 09.07.1993
(51) Int. Cl.: H01J 61/36, H01J 9/26

(54) **STRUCTURE OF SEALING PART OF ARC TUBE AND METHOD OF MANUFACTURING THE SAME**
STRUKTUR VON ABTICHTUNGSTEIL EINER BOGENRÖHRE UND VERFAHREN ZUR HERSTELLUNG DERSELBEN
STRUCTURE DE LA PARTIE DE SCELLEMENT D'UN TUBE A DECHARGE ET PROCEDE DE FABRICATION

(30) Priority: 09.07.1992 JP 20609292; 09.11.1992 JP 32367692; 25.01.1993 JP 2868293
(43) Date of publication of application: 26.04.1995
(73) Proprietor: TOTO LTD., Kitakyushu-shi Fukuoka 802 (JP)
(72) Inventor: NAGAYAMA, Hiroyuki, Toto Ltd, Kita-kyusyu-shi Fukuoka 802 (JP)
(74) Representative: Marsden, John Christopher
(86) International application number: JP9300959
(87) International publication number: WO9401884

(56) References cited:
- EP-A- 0 528 428
- DE-A- 2 032 277
- JP-A- 1 302 652
- JP-A- 2 015 557
- JP-B- 45 030 431

## Description

### Technical Field

The present invention relates to a sealing structure for a light-emitting bulb assembly for use in a metal-vapor discharge lamp such as a mercury-vapor lamp, a metal halide lamp, or a sodium-vapor lamp, or a high-intensity discharge lamp, and a method of manufacturing such a light-emitting bulb assembly.

### Background Art

Metal-vapor discharge lamps include a mercury-vapor lamp, a metal halide lamp, and a sodium-vapor lamp. The mercury-vapor lamp emits light excited from the mercury in a positive column produced in a hot-cathode arc discharge. In the metal halide lamp, a metal halide is evaporated into a metal and a halogen by the heat of a mercury hot-cathode arc discharge to emit light in a color inherent in the metal. The sodium-vapor lamp emits light in yellowish orange at a D line (589.0 nm, 589.9 nm) produced by a hot-cathode arc of a sodium vapor. Heretofore, such metal-vapor discharge lamps have been used as illuminating lamps for gymnasiums and factories, light sources for overhead projectors and color liquid crystal projectors, fog lamps for automobiles, and so on.

The bulbs of metal-vapor discharge lamps were initially made of quartz glass. However, since the quartz glass has poor fade resistance and a large thermal capacity, the metal-vapor discharge lamps cannot be turned on quickly and the individual bulbs have large dimensional variations. Therefore, it has recently been proposed to make bulbs of light-transmissive ceramic.

Generally, a light-emitting bulb assembly for a discharge lamp comprises a bulb made of light-transmissive ceramic in the form of fired alumina or the like, and a closure by which an electrode supported by an electrode support is sealed and fixed in the bulb. To join the closure hermetically to an open end of the bulb, a glass solder is filled in a gap between end and inner surfaces of the open end of the bulb and a confronting surface of the closure, heating the glass solder to melt same, and then cooling and solidifying the melted glass solder.

It is the general practice for the closure to have the same coefficient of thermal expansion as and to be as chemically stable against metal vapor and halogen vapor as the bulb or the electrode support.

When the closure is joined to the bulb by the glass solder, a starting rare gas and a discharging metal component depending on the discharge lamp which incorporates the bulb assembly, e.g., mercury if the discharge lamp is a high-pressure mercury vapor lamp, or a metal halide if the discharge lamp is a metal halide lamp, are sealed in the bulb.

The bulb assembly is turned on, its temperature momentarily increases from the atmospheric temperature to 900°C at which the bulb assembly remains energized stably. High thermal stresses are developed in the bulb assembly due to such a large thermal change and a change in the internal pressure.

When thermal stresses are produced, thermal strains are developed in a portion having a different coefficient of thermal expansion, specifically the closure that is interposed between the bulb and the electrode support, tending to cause the closure to be broken. More specifically, cracks are produced in the closure itself and the glass solder which has lower heat resistance than the light-transmissive ceramic and the closure because of its composition, allowing the discharging metal component to leak out of the bulb. As a result, the bulb assembly is not liable in producing stable light emission, and the service life of the lamp is limited.

In a high-temperature, high-pressure environment in which the temperature and the internal pressure of the bulb assembly are increased, a metal halide (e.g., T1I₃, NaI, or the like) sealed as a discharging metal component is liberated as ions which erode the bulb assembly.

The liberated ions erode the glass solder more quickly because the glass solder has lower erosion resistance than the light-transmissive ceramic and the closure because of its composition. The glass solder is liable to crack also due to the low erosion resistance against the erosion caused by the liberated ions.

Highly pure light-transmissive alumina which is used in the bulb has poor wettability with respect to the glass solder. Therefore, the bonding strength at the boundary between the glass and the bulb is low, tending to produce cracks and a leakage of the sealed gas.

Various arrangements have heretofore been proposed in order to solve the above problems.

Japanese laid-open patent publication No. 1-143132 discloses a technique for brazing an insert having a coefficient of thermal expansion similar to that of alumina to a sealed region of an outer circumferential element of alumina which corresponds to a bulb. According to Japanese laid-open patent publication No. 63-308861, a closure is composed of a central body and an annular body disposed around the central body, and a bulb is joined in solid phase to the closure (the central body and the annular body). Japanese laid-open patent publication No. 63-308861 particularly proposes specific dimensions and compositions of the central body and the annular body which make up the closure. Specified dimensions are also proposed in Japanese laid-open patent publication No. 62-21306.

The disclosed proposals are effective in suppressing a leakage of the discharging metal component from the bulb assembly for thereby keeping reliable light emission and increasing the service life of the lamp.

DE-A-2032277 describes a sealing structure for a bulb in which an electrode core is surrounded by rings of material of varying coefficient of thermal expansion.

Recent years have seen a demand for brighter light emission to achieve higher added values of light-emitting bulb assemblies, and it has been practiced to increase the temperature of a light-emitting bulb assembly up to about 1200°C in excess of the conventional temperature of 900°C in order to attain brighter light emission.

Since the higher bulb temperature leads to corresponding thermal stresses in the bulb assembly, the conventional light-emitting bulb assembly fails to keep sufficiently reliable light emission and have a sufficiently long service life. Specified dimensions of the closure and other parts are not preferable as they pose limitations on the configurations of the light-emitting bulb assembly and also the configurations of the lamp which accommodates the light-emitting bulb assembly.

The present invention has been made in order to solve the above problems. It is an object of the present invention to provide a light-emitting bulb assembly which is highly reliable and has a long service life, and particularly a novel sealing structure for such a light-emitting bulb assembly and a simple method of manufacturing such a light-emitting bulb assembly.

### Disclosure of the Invention

The invention provides a light-emitting bulb having a sealing structure, which includes a closure (303), having a core (304) which serves as an electrode, for sealing an open end (302) of the bulb, said closure including a bulb-side region (303₁) disposed adjacent to the open end of said bulb and made of a compositional ingredient having a coefficient of thermal expansion which is substantially the same as that of the bulb, a core-side region (303ₙ) disposed adjacent to said core and made of a compositional ingredient having a coefficient of thermal expansion which is substantially the same as that of the core, and an intermediate region (303₂ - 303ₙ₋₁) disposed between said bulb-side region and said core-side region and made of a compositional ingredient having compositional proportions adjusted such that the coefficient of thermal expansion thereof varies gradually from the coefficient of thermal expansion of said bulb-side region towards the coefficient of thermal expansion of said core-side region; wherein said bulb-side region and said core-side region comprise a bulb-side region layer and a core-side region layer, respectively, which are independent of each other, and wherein said intermediate region comprises at least one layer whose coefficient of thermal expansion varies gradually from said bulb-side region towards said core-side region; and wherein said at least one layer of the bulb-side region, the intermediate region and said core-side region layer are successively arranged in an axial direction of said bulb.

Preferably, layers of the closure are progressively thicker from the bulb-side region layer toward the core-side region layer.

The bulb should preferably be made of light-transmissive ceramic, particularly highly pure alumina, and the core should preferably be made primarily of tungsten.

The closure may be made of a gradient function material.

The above sealing structure may be manufactured by a method given below.

A method of manufacturing a light-emitting bulb assembly including a closure having a core which serves as an electrode and sealing an open end of a light-transmissive bulb, comprises the steps of:
(a) preparing, from a fine powder of a light-transmissive bulb ingredient and a fine powder of a core ingredient, a bulb ingredient suspension in which the light-transmissive bulb ingredient is greater than the core ingredient, a core ingredient suspension in which the core ingredient is greater than the light-transmissive bulb ingredient, and at least one intermediate suspension in which the light-transmissive bulb ingredient and the core ingredient have compositional proportions lying between those of the bulb ingredient suspension and the core ingredient suspension;
(b) forming an unfired laminated body composed of an unfired bulb-side region layer to be disposed adjacent to the light-transmissive bulb and formed from the bulb ingredient suspension, an unfired core-side region layer to be disposed adjacent to the core and formed from the core ingredient suspension, and at least one unfired intermediate region layer disposed between the unfired bulb-side region layer and the unfired core-side region layer and formed from the at least one intermediate suspension; and
(c) firing the unfired laminated body.

The step (b) may comprise the steps of:
(d) pouring the bulb ingredient suspension into a cavity defined in a mold assembly composed of a plurality of joined molds each made of a porous material, causing a solvent of the bulb ingredient suspension to penetrate into the mold assembly, and thereafter discharging an excessive amount of the bulb ingredient suspension from the mold assembly, thereby forming the bulb-side region layer on an inner surface of the cavity;
(e) thereafter, successively pouring the at least one intermediate suspension and the core ingredient suspension onto an inner surface of the bulb-side region layer, allowing solvents of the at least one intermediate suspension and the core ingredient suspension to penetrate into the mold assembly, and thereafter discharging excessive amounts of the at least one intermediate suspension and the core ingredient suspension from the mold assembly, thereby forming a molded laminated body; and
(f) separating the molds from each other, thereby releasing the molded laminated body as the unfired laminated body.

Alternatively, the step (b) may comprise the steps of producing green sheets respectively from the core ingredient suspension, the at least one intermediate suspension, and the bulb ingredient suspension, and successively winding the green sheets around the core, thereby forming the unfired laminated body.

In the above sealing structure, the core comprises a conductive core made of tungsten or the like, and the closure hermetically joined in solid phase to the opening of the bulb comprises a fired laminated body composed of a core-side region layer, at least one intermediate region layer, and a bulb-side region layer which are successively arranged from the conductive core toward the bulb. The core-side region layer includes at least 50 % by volume of an ingredient of the conductive core, and the bulb-side region layer includes at least 80 % by volume of an ingredient of light-transmissive ceramic. The intermediate region layer between the core-side region layer and the bulb-side region layer includes light-transmissive ceramic having a volume ratio which is progressively closer to the volume ratio of the light-transmissive ceramic of the bulb-side region in a direction toward the bulb-side region, and also includes the ingredient of the core having a volume ratio which is progressively closer to the volume ratio of the ingredient of the core in the core-side region layer in a direction toward the core-side region layer.

In each of the layers of the closure, a network structure of crystals is formed between common ingredients by firing, thereby integrally joining the ingredients. A firing process for reducing surface energy is applied to the joining of the core and the opening of the bulb to each other. Impurities such as of glass are often added in a small amount in an effort to accelerate the firing process.

More specifically, each of the layers traps the powder of the ingredient of the conductive core, and the ingredient of the light-transmissive ceramic forms a solid solution and is crystallized. Adjacent layers are integrally joined to each other in solid phase as the ingredient of the light-transmissive ceramic in the layers forms a solid solution and is crystallized at the mating surfaces of the layers. The conductive core and the core-side region layer are also integrally joined to each other in solid phase because the ingredient of the light-transmissive ceramic in the core-side region layer is crystallized in contact with the core, forming a glassy substance which fills in its grain boundaries, and also because the ingredient of the conductive core is contained in both the core and the core-side region layer. Furthermore, the bulb-side region layer and the bulb are also integrally joined to each other in solid phase because the ingredient of the light-transmissive ceramic in the bulb-side region layer is crystallized in contact with the bulb, forming a glassy substance which fills in its grain boundaries, and also because the ingredient of the light-transmissive ceramic is contained in both the bulb-side region layer and the bulb.

Therefore, the closure after it has been fired is firmly bonded to the conductive core, making it possible to seal a main electrode. Additionally, the closure after it has been fired makes it possible to hermetically seal the opening of the bulb through the formation of a glass phase in the grain boundaries of the ingredient of the light-transmissive ceramic in the bulb-side region layer and the bulb.

In addition, the distribution of coefficients of thermal expansion from the conductive core through the core-side region layer, the intermediate region layer, and the bulb-side region layer to the bulb is a gradient distribution ranging from the coefficient of thermal expansion of the conductive core to the coefficient of thermal expansion of the bulb.

In the method of manufacturing the sealing structure, when the closure to be hermetically joined in solid phase to the opening of the bulb which is made of light-transmissive ceramic is to be fired, an unfired core-side region layer, an unfired intermediate region layer, and an unfired bulb-side region layer are successively stacked on a core made of a conductive material, thereby forming an unfired laminated body.

The unfired core-side region layer, the unfired intermediate region layer, and the unfired bulb-side region layer which are successively stacked are formed from a core ingredient suspension including a powder of a conductive material ingredient or a core ingredient and a powder of a light-transmissive ceramic ingredient or a bulb ingredient, with at least 50 % by volume of the conductive material ingredient, a bulb ingredient suspension including both powders with at least 80 % by volume of the light-transmissive ceramic ingredient, and a plurality of intermediate suspensions including both powders with the volume ratio of the light-transmissive ceramic ingredient being progressively increased to a value close to 100 % and the volume ratio of the conductive material ingredient being progressively reduced from 100 %.

To successively deposit the unfired core-side region layer, the unfired intermediate region layer, and the unfired bulb-side region layer on an outer surface of the core, they are deposited in a descending order of volume ratios of the conductive material ingredient, thereby forming the unfired laminated body. Thereafter, the unfired laminated body is disposed at the opening of the bulb so as to position the main electrode connected to the core in the bulb, and then fired.

After the laminated body has been fired, since the light-transmissive ceramic ingredient forms a solid solution and is crystallized, trapping the powder of the core ingredient, in each of the layers, the fired closure is of an integral structure achieved by the formation of a solid solution of and crystallization of the light-transmissive ceramic ingredient between adjacent ones of the layers. The fired closure is firmly bonded to the core, making it possible to seal the main electrode, through the formation of a glass phase in the grain boundaries of the light-transmissive ceramic ingredient in the core-side region layer while it is being held in contact with the core, and also through the coexistence of the conductive core ingredient. The fired closure also makes it possible to hermetically seal the opening of the bulb through the formation of a glass phase in the grain boundaries of the light-transmissive ceramic ingredient in the bulb-side region layer and the bulb.

Moreover, the distribution of coefficients of thermal expansion from the core through the core-side region layer, the intermediate region layer, and the bulb-side region layer to the bulb is a gradient distribution ranging from the coefficient of thermal expansion of the core to the coefficient of thermal expansion of the bulb.

### Brief Description of the Invention

Original figures 1,2, 4, 5(a) through 5(c), 15, 20-22, and 23(a) through 23(f), were deleted during the examination procedure.
Fig. 3 is a diagram showing a process of manufacturing the closure of the light-emitting bulb assembly;
Fig. 6 is a diagram showing a process of manufacturing a closure of a light-emitting bulb assembly according to a first embodiment of the present invention;
Fig. 7 is a perspective view of an unfired molded body which will be fired into the closure;
Figs. 8(a) and 8(b) are perspective views of a mating mold assembly used to produce the closure;
Fig. 9 is a perspective view of the mating mold assembly with an auxiliary member attached thereto;
Figs. 10(a) and 10(b) are views illustrative of a process of manufacturing the closure;
Fig. 11 is a cross-sectional view of the closure which is molded in the mating mold assembly;
Figs. 12(a) and 12(b) are diagrams showing composition distributions of the closure;
Fig. 13 is a cross-sectional view of the unfired closure with an electrode attached thereto;
Fig. 14 is a cross-sectional view of the closure as it is mounted in a bulb;
Fig. 16 is a cross-sectional view of a light-emitting bulb assembly according to a second embodiment of the present invention;
Fig. 17 is a diagram showing a process of preparing a slip for a closure of the light-emitting bulb assembly;
Figs. 18(a) through 18(e) are diagram showing a slip-casting process;
Fig. 19 is a cross-sectional view of a light-emitting bulb assembly according to a modification of the third embodiment;
Fig. 24 is a cross-sectional view of a light-emitting bulb assembly according to a third embodiment of the present invention;
Fig. 25 is a diagram showing respective slips used to manufacture the light-emitting bulb assembly;
Fig. 26 is a perspective view of a tubular pipe used to manufacture the light-emitting bulb assembly;
Figs. 27(a) and 27(b) are views showing a process of manufacturing the light-emitting bulb assembly;
Fig. 28 is a cross-sectional view of a light-emitting bulb assembly according to a fourth embodiment of the present invention;
Figs. 29(a) through 29(e) are views showing slips used to manufacture a closure of the light-emitting bulb assembly and a process of manufacturing the closure; and
Figs. 30(a) through 30(d) are views showing a modification of the process of manufacturing the closure.

### Best Mode For Carrying Out the Invention

Preferred embodiments of light-emitting bulb assemblies according to the present invention will be described below with reference to the drawings.

The main electrodes 3 are in the form of tungsten coils, respectively, which are supported by respective support shafts 4 of tungsten which extend through the closure 2a.

The end of the bulb with the electrode holding hole 1b has a slender introduction tube 1c for entering a starting rare gas metal and various discharging material amalgams. The slender introduction tube 1c has an open end sealed by a sealant 1d of a cermet of alumina or a metal such as nickel or the like.

A process of manufacturing the light-emitting bulb assembly will be described below.

Synthesis of a fine powder of alumina which will be used as a material of the bulb and the closure will first be described below.

To synthesize a fine powder of alumina, an aluminum salt which will become alumina having a purity of 99.98 mol % or more when thermally decomposed is used as a starting material.

An aluminum salt for synthesizing such highly pure alumina may be ammonium alum or aluminum ammonium carbonate hydroxyside (NH₄AlCO₃(OH)₂).

The aluminum salt is then weighed, dissolved together with a dispersing agent in distilled water, thus producing a suspended aqueous solution, and then dried by a spray drying process. The dried aluminum salt is thereafter thermally decomposed, thereby producing a fine powder of alumina only. The dried aluminum salt is thermally decomposed at 900 ∼ 2000°C, e.g., 1050°C, in the atmosphere for 2 hours. The fine powder of alumina produced by the spray drying process and the thermal decomposition has an average particle diameter ranging from 0.2 to 0.3 µm and a purity of 99.99 mol % or higher. The fine powder of alumina is thus prepared. The synthesized fine powder of alumina is obtained as a secondary aggregate of fine powder of alumina having the above particle diameter, the secondary aggregate being of a size greater than the above particle diameter.

As another material of the closure than alumina, a fine powder of tungsten is prepared which has a purity of 99 mol % or higher and an average particle diameter of about 0.5 µm.

The bulb is manufactured as follows:

To the synthesized fine powder of alumina (secondary aggregate), there is added an organic binder which is composed primarily of an acrylic thermoplastic resin. The fine powder of alumina and the added organic binder are mixed with each other in a wet manner using an organic solvent such as of alcohol, benzene, or the like by a plastic (nylon) ball mill for about 24 hours, so that the fine powder of alumina and the organic binder are sufficiently wetted. The mixture is then distilled and dried, thereby removing the solvent, and kneaded into a compound having a desired viscosity ranging from 50,000 to 150,000 cps.

The organic binder is a mixture of an acrylic thermoplastic resin, paraffin wax, and atactic polypropylene. The total amount of the organic binder with respect to 100 g of the fine powder of alumina is 25 g.

The ingredients of the organic binder are of the following proportions, and adds up to the total amount (25 g) of the organic binder:

| | |
|---|---|
| Acrylic thermoplastic resin | 20 ∼ 23 g (preferably, 21.5 g) |
| Paraffin wax | 3 g or less (preferably, 2.0 g) |
| Atactic polypropylene | 2 g or less (preferably, 1.5 g) |

The mixture is distilled and dried at 130°C for 24 hours, and thereafter kneaded at 130°C by a roll mill of alumina into the compound having the desired viscosity.

Subsequently, the compound is injection-molded into a molded body. The molded body is heated in a nitrogen atmosphere up to a temperature at which the organic binder of the acrylic thermoplastic resin, etc. is thermally decomposed and fully carbonized, so that the molded body is degreased. The specific upper limit temperature up to which the molded body is to be heated in this initial heat treatment may be determined depending on the capability of a heat treatment furnace used and the temperature at which the organic binder is thermally decomposed. In this embodiment, the molded body is heated from room temperature (20°C) to 450°C in 72 hours. Other processing conditions are given below. While the molded body is being heated up to 450°C, it is kept under a constant pressure.

| | |
|---|---|
| Processing pressure | 1 ∼ 8 kg/cm² (optimum pressure: 8 kg/cm²) |
| Time required to heat the molded body from 20°C to 450°C | 72 hours or shorter |

In the initial heat treatment, the added organic binder composed of an acrylic thermoplastic resin, paraffin wax, and atactic polypropylene is thermally decomposed and carbonized, so that the molded body is degreased.

Then, the molded body (degreased body) is fired in the atmosphere by subsequent heat treatment under conditions given below, thereby producing a fired body. The molded body is heated at a rate of 100°C/hour.

| | |
|---|---|
| Processing temperature | 1200 ∼ 1300°C (optimum temperature: 1235°C) |
| Time during which the molded body is kept at the processing temperature | 0 ∼ 4 hours (optimum time: 2 hours). |

The molded body is fired by the subsequent heat treatment in the temperature range of from 1200 to 1300°C for the reasons that the density of the fired molded body will be 95 % or more of the theoretical density for being subject to subsequent hot isostatic pressing, and large crystals will not be produced in the fired body. If the molded body were fired at a temperature lower than 1200°C, then the density of the fired molded body would be less than 95 % of the theoretical density and the molded body would not be subject to hot isostatic pressing. If the molded body were fired at a temperature higher than 1300°C, then the fired body would have large crystals at a greater frequency, and would not be sufficiently strong.

The molded body is thus fired after it is degreased by the initial heat treatment and the subsequent heat treatment. The volume of the molded body thus fired is reduced such that the volume of the molded body is 82.5 % of the volume of the molded body before it is fired. The packing ratio of the fired body is about 100 % (bulk density: 3.976). Until the subsequent heat treatment is completed, the carbonized material which has been modified in the initial heat treatment is completely burned away.

Thereafter, the fired body is subjected to hot isostatic pressing in an argon atmosphere or an argon atmosphere which contains 20 vol. % or less of oxygen under conditions given below. At this time, the fired body is heated at a rate of 200°C/hour. The fired body thus pressed exhibits a light-transmitting ability.

| | |
|---|---|
| Processing temperature | 1200 ∼ 1250°C (optimum temperature: 1230°C) |
| Processing pressure | 1000 ∼ 2000 atm (optimum pressure: 1000 atm) |
| Processing time | 1 ∼ 4 hours (optimum processing time: 2 hours) |

The fired body is subjected to hot isostatic pressing in the above temperature range and pressure range in order to achieve a desired high light-transmitting ability and improve its mechanical strength to avoid damage during the hot isostatic pressing. If the hot isostatic pressing were carried out at a temperature lower than 1200°C or under a pressure lower than 1000 atm, then though the fired body would be rendered light-transmissive, but the obtained light-transmitting ability would be low. If the hot isostatic pressing were carried out at a temperature in excess of 1250°C, then abnormal grain growth would be accelerated, inviting a reduction in the mechanical strength and the light-transmitting ability. If the hot isostatic pressing were carried out under a pressure in excess of 2000 atm, then stresses would concentrate in regions where bores and flaws, even if extremely small, are located in the fired body, tending to cause the fired body to crack in those regions.

Thereafter, the ends of the fired body are ground by a diamond grinding wheel (not shown) to remove edges, thereby completing the light-transmissive bulb of alumina.

The inner and outer surfaces of the bulb thus produced are then ground by a brush with a diamond grinding grain having a particle diameter of 0.5 µm until the bulb 1F will have a wall thickness of 0.2 mm or less. Surface irregularities are thus removed to prevent light from being scattered by the surfaces of the bulb and improve a liner transmittance thereof.

The completed bulb made of light-transmissive alumina has smaller crystal grain diameters than general light-transmissive ceramics which are produced by firing alumina with a sintering additive of MgO or the like for greater crystal grains.

The bulb fabricated from highly-pure alumina has a light-transmitting ability while having small crystal grain diameters different from those of general light-transmissive ceramics for the following reasons:

Since only a small amount of oxide such as MgO or the like mixed as an impurity (a total of 0.01 mol % or less at maximum) is contained in the powder of alumina, the impurity forms in its entirety a solid solution with alumina, producing almost no grain boundary phase. Therefore, the effect of a grain boundary phase which is responsible for diffusing light in general light-transmissive alumina is eliminated, resulting in an increase in the linear transmittance with respect to visible light.

Furthermore, the following considerations are taken into account:

If it is assumed that all the crystal grains and crystallites have a circular cross section, then a crystal grain having a diameter D and made up of n crystallites each having a diameter d satisfies the following equation ①:${\text{n = (D/d)}}^{\text{2}}$

The value of n calculated according to the above equation can be converted into crystallite boundaries contained in the cross section of one crystal grain.

The lattice constants of various light-transmissive aluminas obtained from highly pure alumina (having average particle diameters of 0.72, 0.85, 0.99, 1.16, 1.35, 1.52 µm) were determined using an X-ray diffraction apparatus, and the diameters d of the crystallites of the light-transmissive aluminas having the above average particle diameters were calculated from diffraction peaks (012) according to the Scherrer's equation which relates the diameter d of a crystallite to the width of a diffraction line. As a result, it was found that the diameters d of the crystallites were constant irrespective of the sizes of the crystal grains. The Scherrer's equation is given in P. Gallezot, "Catalysis, Science and Technology", vol. 5 p. 221, Springer-Verlag (1984), and P. Scherrer, "Gottinger Nachrichen", 2, 98 (1918).

It can therefore be seen from the above equation (1) that the smaller the diameters D (average particle diameter) of the crystal grains, the fewer the crystallite boundaries in one crystal grain.

Generally, it is considered that when light is applied to a polycrystalline material such as of ceramic, the light is diffused by surfaces where refractive indexes are not continuous, i.e., regions where the arrangement of atoms is discontinuous. Since a crystallite boundary in a crystal grain is nothing but such a region where the arrangement of atoms is discontinuous, it causes a diffusion of light. Consequently, the fewer the crystallite boundaries in a crystal grain, i.e., the smaller the diameter D of a crystal grain, the smaller the effect of the crystallite boundaries which are responsible for diffusing light, giving rise to an increase in the linear transmittance with respect to visible light.

The closures are manufactured as described below. A process of manufacturing the closures will be described below with reference to Fig. 3.

First, a vehicle to be used to suspend therein the fine powder of alumina (secondary aggregate) synthesized as described above and the fine powder of tungsten is prepared from various organic materials given in Table 1 below (step 1). To prepare the vehicle, the organic materials are weighed and uniformly mixed by a mixer.

**Table 1**

| Ingredients | Volume ratio |
|---|---|
| α-terpineol | 50 |
| butyl acetate carbitol | 20 |
| ethyl cellulose | 3 |
| polyvinyl butyral | 7 |
| ethanol | 10 |

The fine powder of alumina, the prepared vehicle, an organic solvent (butyl diphthalate), and a dispersing agent (ammonium carboxylic acid) are mixed at volume ratios given in Table 2, below, and kneaded into an alumina slurry by three rolls (step 2).

**Table 2**

| Ingredients | Volume ratio |
|---|---|
| fine powder of alumina | 64 |
| vehicle | 32 |
| butyl diphthalate | 3.5 |
| ammonium carboxyl acid | 0.5 |

The fine powder of tungsten, the prepared vehicle, an organic solvent (butyl diphthalate), and a dispersing agent (ammonium carboxylic acid) are mixed at volume ratios given in Table 3, below, and kneaded into a tungsten slurry by three rolls (step 2).

**Table 3**

| Ingredients | Volume ratio |
|---|---|
| fine powder of tungsten | 82 |
| vehicle | 15 |
| butyl diphthalate | 2.6 |
| ammonium carboxyl acid | 0.4 |

Using the alumina slurry prepared at the volume ratios given in Table 2 and the tungsten slurry prepared at the volume ratios given in Table 3, eight slurries composed of tungsten and alumina mixed at volume ratios (tungsten/ alumina) given in Table 4, below, are prepared (step 3).

**Table 4**

| Slurries | Volume ratio (tungsten/alumina) |
|---|---|
| 1st layer slurry | 80/20 |
| 2nd layer slurry | 60/40 |
| 3rd layer slurry | 40/60 |
| 4th layer slurry | 30/70 |
| 5th layer slurry | 20/80 |
| 6th layer slurry | 10/90 |
| 7th layer slurry | 5/95 |
| 8th layer slurry | 3/97 |

Each of the mixed slurries thus prepared is sufficiently mixed such that alumina and tungsten are uniformly dispersed, and thereafter debubbled (step 4). More specifically, each of the mixed slurries is put in a resin container in a vacuum desiccator, and air in the vacuum desiccator is drawn out by a vacuum pump for a few tens of minutes (e.g., about 20 minutes) while the slurry in the resin container is being stirred by a magnet stirrer or the like. While the slurry is being debubbled in vacuum, the organic solvent is partly volatilized to achieve a slurry viscosity of 30,000 cP.

The mixed slurries shown in Table 4 are applied in a descending order of volume ratios of tungsten, i.e., from the first layer slurry to the eighth layer slurry. A laminated body 20a as a precursor of each of the closures 2a is thus formed around the support shafts 4 (step 5). The mixed slurries are applied to and deposited on the outer circumferential surface of each of the support shafts 4 in the order from the first layer slurry to the eighth layer slurry by coating and drying each of the slurries successively from the first layer slurry.

In this manner, an innermost layer composed of the first layer slurry is formed in a core-side region of the closure which is located adjacent to the core, a plurality of intermediate layers composed of the second through seventh layer slurries are formed in an intermediate region of the closure, and an outermost layer composed of the eighth layer slurry is formed in a bulb-side region of the closure which is located adjacent to the open end of the bulb.

Then, the laminated body is heated to 600°C for 10 hours in a moisture-containing hydrogen reducing atmosphere, so that the laminated body is degreased (step 6). Specifically, when the laminated body is heated, the organic materials and organic solvent which are contained in the vehicle that were added when the slurries were prepared are thermally decomposed and carbonized, thereby degreasing the formed body.

The degreased laminated body is subsequently heated to 1800°C for 2 hours in a vacuum atmosphere and fired (step 7). The closure 2a is now obtained as the fired laminated body. Until this subsequent heat treatment is completed, the carbonized materials modified in the above initial heat treatment are fully burned away.

In each of the layers of the closures 2a a network structure of crystals is formed between common ingredients by firing, thereby integrally joining the ingredients. A firing process for reducing surface energy is applied to the joining of the support shafts 4 and the surfaces of the electrode holding holes 1a, 1b of the bulb to each other. Impurities such as of glass are often added in a small amount in an effort to accelerate the firing process.

More specifically, in the firing process, the alumina forms a solid solution and is crystallized, trapping the powder of tungsten, in each layer of the laminated body. Adjacent layers of the laminated body are integrally joined to each other in solid phase as the alumina in the layers forms a solid solution and is crystallized at the mating surfaces of the layers. The support shaft 4 and the innermost layer composed of the first layer slurry are also integrally joined to each other in solid phase because alumina in the innermost layer is crystallized in contact with the support shaft 4, forming a glassy substance in its grain boundaries, and also because tungsten is contained in both the support shaft 4 and the innermost layer. As a result, the fired closure 2a is strongly bonded to the support shafts 4 which support the main electrodes 3, hermetically sealing and securing the support shafts 4 and hence the main electrodes 3 in the bulb.

The distribution of coefficients of thermal expansion from the support shaft 4 through the innermost layer and the intermediate layers to the outermost layer is a gradient distribution ranging from the coefficient of thermal expansion of the support shaft 4 (the coefficient of thermal expansion of tungsten) to a coefficient of thermal expansion which is close to the coefficient of thermal expansion of the bulb (the coefficient of thermal expansion of alumina), based on the composition distributions thereof.

After the support shafts 4 have been sealed and secured, the outer circumferential surfaces of the outermost layers of the closures 2a are cut or ground so as to fit in the electrode holding holes 1a, 1b in the bulb (step 8). The closures are now completed, and the manufacturing process is ended.

Assembling the completed closures 2a into the bulb and fabrication of the light-emitting bulb assembly 1 will be described below.

First, the closure which has been fired and machined on its outer circumferential surface is fitted in the electrode holding hole in the bulb, bringing the outer circumferential surface of the closure 2A into contact with the inner circumferential surface of the electrode holding hole. Thereafter, an infrared radiation or high-output laser beam is locally applied to the contacting surfaces to heat them.

The localized heating causes the alumina in the outermost layer composed of the eighth layer slurry of the closure and the alumina in the bulb to be fired and crystallized, and also causes grain boundaries in the joined surfaces to be embedded by a glass phase that is primarily of a structure of spinel, garnet or the like. The closure and the bulb are therefore joined in solid phase to each other. As a consequence, the closure and the bulb are hermetically secured to each other by the formation of a glass phase in the grain boundaries of alumina in the outer-most layer and the bulb.

The bulb is now ready for being filled with a starting rare gas metal and a discharging material.

Then, an amalgam of a given starting rare gas metal and a discharging material (an alloy of Sn, Na-T1-In, Se-Na, Dy-T1, or a halide of each of the metals) is introduced through the slender introduction tube 1c into the bulb whose ends have been sealed, and thereafter the slender introduction tube 1c is sealed by the sealant 1d.

Since the closures and the bulb are integrally joined in solid phase to each other without use of soldering glass which has heretofore been relied upon, the materials which have been sealed in the bulb are reliably prevented from leaking out.

The bulb with the main electrodes mounted therein are generally incorporated in an outer tube of a high-pressure discharge lamp such as a metal halide lamp or the like.

A first embodiment of the present invention will be described below. Closures of a light-emitting bulb assem-

The materials of the closure 2a (see Fig. 14) according to the second embodiment are, as above, a fine powder of highly pure alumina synthesized by drying an aqueous solution of suspended aluminum salt according to a spray drying process and then thermally decomposing the aluminum salt, and a fine powder of highly pure tungsten.

A process of manufacturing the closure 2a according to the first embodiment will be described below with reference to Fig. 6.

As shown in Fig. 6, eleven slurries with the following volume ratios of tungsten and alumina (tungsten/ alumina) are prepared from a fine powder of alumina and a fine powder of tungsten (step 1):
1st slurry: tungsten/alumina = 100/0
2nd slurry: tungsten/alumina = 90/10
3rd slurry: tungsten/alumina = 80/20
4th slurry: tungsten/alumina = 70/30
5th slurry: tungsten/alumina = 60/40
6th slurry: tungsten/alumina = 50/50
7th slurry: tungsten/alumina = 40/60
8th slurry: tungsten/alumina = 30/70
9th slurry: tungsten/alumina = 20/80
10th slurry: tungsten/alumina = 10/90
11th slurry: tungsten/alumina = 0/100

The above slurries are prepared as follows: First, the fine powder of alumina and the fine powder of tungsten are weighed such that their volume ratios are of the above numerical values, and a dispersing agent of ammonium carboxylic acid and distilled water are added to the weighed powders. They are then mixed with each other in a wet manner by a ceramic (alumina) ball mill for about 24 hours, so that the fine powders of alumina and tungsten are uniformly present in the solvent while breaking up excessive aggregates.

The ratio (volume ratio) at which the dispersing agent of ammonium carboxylic acid is added to the fine powders in each of the slurries is 2 g with respect to 100 g of the total fine powders in each of the slurries.

Then, each of the slurries is debubbled (step 2). Specifically, each of the slurries taken from the ball mill is put in a resin container in a vacuum desiccator, and air in the vacuum desiccator is drawn out by a vacuum pump for a few tens of minutes (e.g., about 20 minutes) while the slurry in the resin container is being stirred by a magnet stirrer or the like.

Thereafter, a desired molded body 20a shown in Fig. 7 is produced using a mating mold assembly 10 shown in Fig. 8(a) according to a process described below. The ratio of vertical and horizontal dimensions of the molded body 20a and the closure 2a shown in Figs. 7 and 10(a), 10(b) is not 1 : 1 for illustrative purpose.

The mating mold assembly 10 comprises a pair of symmetric molds 11a, 11b each made of a porous inorganic material such as plaster or the like or a porous resin with minute pores which has substantially the same function as plaster. The molds 11a, 11b are joined to each other, defining a slurry pouring space 13 between mating surfaces of the molds 11a, 11b as shown in Fig. 8(a).

As shown in Fig. 8(b), the molds 11a, 11b have respective grooves (cavities) 13a, 13b defined in the respective mating surfaces 15a, 15b and curved in the vicinity of lower mold ends. The grooves 13a, 13b are cut in the respective mating surfaces 15a, 15b by an end mill having a spherical cutter on its distal end. Alternatively, the grooves 13a, 13b may initially be formed in the respective mating surfaces 15a, 15b.

Then, the debubbled slurries are poured in a descending order of contents of alumina, i.e., from the eleventh slurry to the first layer slurry, into the slurry pouring space 13 of the mating mold assembly 10 (step 3).

Specifically, as shown in Fig. 9, a cylindrical member 17 is placed on the upper surface of the mating mold assembly 10, and the eleventh slurry, which is of an amount greater than the volume of the slurry pouring space 13, is poured into the cylindrical member 17. An annular piece of clay 19 is applied to the lower end of the cylindrical member 17 to provide a seal between the lower surface of the cylindrical member 17 and the upper surface of the mating mold assembly 10. The clay may be replaced with rubber.

After the eleventh slurry has been poured into the slurry pouring space 13, the poured eleventh slurry is left for a predetermined period of time. During this time, the solvent (distilled water) of the eleventh slurry is drawn into the pores of the porous molds 11a, 11b by capillary action. Accordingly, a powder (alumina powder in the eleventh slurry) bounded by the dispersing agent of ammonium carboxylic acid is uniformly deposited on the wall surface of the slurry pouring surface 13, forming a thin layer 11S thereon as shown in Figs. 10(a) and 10(b).

The period of time during which the poured eleventh slurry is left after the eleventh slurry has been poured into the slurry pouring space 13 governs the thickness of the thin layer 11S. The period of time during which the poured eleventh slurry is left is experimentally determined so that the formed thin layer 11S has a predetermined value. The period of time during which the poured eleventh slurry is left and the slurry pouring space 13 are determined also in view of volume shrinkage after firing. The period of time during which the poured eleventh slurry is left according to this embodiment is adjusted so that the formed thin layer 11S has a predetermined value.

While the poured eleventh slurry is being left, a negative pressure may be maintained outside of the molds for forcibly drawing the solvent of the slurry out of the molds. This allows the poured eleventh slurry to be left for a shorter period of time, permits the slurry to be directly debubbled through the molds, and also makes it possible to increase the filling ratio by strongly drawing the solvent.

After the poured eleventh slurry has been left for the predetermined period of time, the eleventh slurry remaining inside the cylindrical member 17 and on the inner surface of the thin layer 11S is discharged. Then, the tenth slurry is poured, left for a predetermined period of time, and discharged. Thereafter, the ninth through first slurries are also poured, left for a predetermined period of time, and discharged. After the eleventh through first slurries are repeatedly poured, left for a predetermined period of time, and discharged, the powders in the slurries (the power of alumina alone, the powder of mixed alumina and tungsten, and the powder of tungsten alone) are uniformly deposited in layers, forming thin layers 11S, 10S, 9S, ···, 1S successively on the wall surface of the slurry pouring space 13. These thin layers 11S, 10S, 9S, ···, 1S jointly form a molded body 20a as a precursor of the closure 2a.

Figs. 12(a) and 12(b) are diagrams showing the relationship between volume ratios of tungsten and alumina in each of the thin layers. As shown in Figs. 12(a) and 12(b), the molded body 20a is of such composition distributions that the volume ratio of alumina increases from 0 % up to 100 % from the central thin layer 1S toward the outer thin layers as shown in Fig. 12(b), and the volume ratio of tungsten decreases from 100 % to 0 % from the central thin layer 1S toward the outer thin layers as shown in Fig. 12(a). The thin layers 2S ∼ 10S are disposed around and covers the central layer 1S.

When the cycles of pouring, leaving for a predetermined period of time, and discharging the eleventh through first slurries are completed, the mating mold assembly 10 is separated, releasing the molded body 20a shaped as shown in Fig. 7. The molded body 20a is dried until the solvent is thoroughly removed therefrom (step 4).

Thereafter, the molded body 20a is heated to 600°C for 10 hours in a moisture-containing hydrogen reducing atmosphere, so that the molded body 20a is degreased and temporarily fired (step 5). Specifically, when the molded body 20a is heated, the dispersing agent which was added when the slurries were prepared is thermally decomposed, thereby degreasing the molded body 20a.

Then, as shown in Fig. 13, support holding holes 21a, 21b are defined respectively in the opposite ends of the molded body 20a, and a support shaft 4 which supports a main electrode 3 is fitted in the support holding hole 21a that is defined in the distal end of the central layer 1S, and a shaft 5 of tungsten is fitted in the support holding hole 21b, thereby setting the main electrode 3 (step 6).

The molded body 20a with the main electrode 3 set is subsequently heated to 1500°C for 2 hours in a vacuum atmosphere, so that the molded body 20a is fired (step 7). The closure 2A is now obtained as the fired molded body 20a. Until this subsequent heat treatment is completed, the carbonized materials modified when the molded body is degreased are fully burned away.

In the firing process, the thin layers of the molded body 20a are integrally joined in solid phase as with the laminated body 20 according to the preceding embodiment. The support shaft 4, the shaft 5, and the thin layer 15 are also integrally joined in solid phase by volume shrinkage upon firing and coexistence of tungsten. As a result, the fired closure 2a is firmly bonded to the support shaft 4 which supports the main electrode 3 and the shaft 5, hermetically sealing and securing the support shaft 4 and the main electrode 3. The closure 2a is now completed, and the process of manufacturing same is completed in its entirety.

The outside diameter of the fired closure 2a is determined by the diameter of the slurry pouring space 13 which takes into account volume shrinkage upon firing. Therefore, the fired closure 2a is not required to be machined at its outer circumferential surface.

The distribution of coefficients of thermal expansion from the support shaft 4 through the thin layers 2S through 9S to the thin layer 10S is a gradient distribution ranging from the coefficient of thermal expansion of the support shaft 4 (the coefficient of thermal expansion of tungsten) to the coefficient of thermal expansion of the bulb (the coefficient of thermal expansion of alumina), based on the composition distributions thereof.

As shown in Fig. 14, the completed closure 2a is fitted in the electrode holding hole 1a in the bulb, and then an infrared radiation or high-output laser beam is locally applied to the contacting surfaces of the closure 2a and the bulb IF to heat them.

The localized heating causes the alumina in the thin layer 10S of the closure 2a and the alumina in the bulb to form a glass phase in the grain boundaries in the joined surfaces. The closure 2a and the bulb are therefore joined in solid phase to each other. As a consequence, the closure 2a and the bulb IF are hermetically secured to each other. Then, a starting rare gas metal and a discharging material are filled in the bulb 1F. The light-emitting bulb assembly shown in Fig. 14 is now completed.

The light-emitting bulb assembly with the closure 2a was measured for its energization service life when repeatedly turned on and off. As a result, it was found that the light-emitting bulb assembly with the closure 2a had very high durability. The light-emitting bulb assembly with the closure 2a has increased resistance against thermal stresses because the closure 2a has a gradient coefficient of thermal expansion that is closer to the coefficient of thermal expansion of either the support shaft 4 having the main electrode 3 or the bulb toward the support shaft 4 and the bulb 1F. Because of such increased resistance against thermal stresses, the light-emitting bulb assembly is capable of highly reliable light emission and has a long service life. The light-emitting bulb assembly can also be made available with ease.

The light-emitting bulb assembly with the closure 2a also offers the following advantages:

Since the volume ratio of alumina is 100 % in the thin layer 11S which is exposed in the bulb in supporting the main electrode 3 in the bulb, i.e., the thin layer 11S is an insulation, back arcs from the main electrode 3 can be avoided for more stable energization of the light-emitting bulb assembly.

Because the main electrode 3 and the shaft 5 which serves as an external terminal are hermetically sealed by the thin layer (central layer) 1S whose volume ratio of tungsten is 100 %, a desired voltage can be applied to the main electrode 3 without fail.

In addition, as the thin layers are formed by pouring slurries, it is possible to uniformize the thicknesses of the thin layers for reliably maintaining composition distributions in the layers and a gradient distribution of coefficients of thermal expansion.

The present invention is not limited to this embodiment, but various changes and modifications may be made therein without departing from the scope of the present invention.

The materials of the bulb and the closure 2a include a fine powder of alumina whose purity is 99.99 mol % or higher in the above embodiment. However, insofar as the bulb has practical linear transmittance (linear transmittance with respect to light having a wavelength ranging from 380 to 760 nm), the material is not limited to such a fine powder of alumina.

For example, the bulb may be in the form of a fired body composed primarily of an oxide such as alumina, magnesia, zirconia, or yttria and a nitride such as aluminum nitride, with a compound (sintering additive) added for suppressing abnormal grain growth and accelerating firing. The closures 2a may be fabricated using the same fine powder of ceramic as the bulb thus produced. More specifically, the bulb may be made of a fine powder of alumina having a purity of 99.2 mol % and an average particle diameter ranging from 0.3 to 1.0 µm, and the closures 2a may be made of such a fine powder of alumina and a fine powder of tungsten.

While the materials of the closures 2a include a fine powder of tungsten in the above embodiments, the materials of the closures 2a may be modified depending on the material of the support shaft 4 which serves as a core. For example, if the support shaft 4 is made of niobium, then the materials of the closures 2, 2a may include a fine powder of niobium.

The bulb may be of any of various shapes. For example, rather than having the larger-diameter electrode holding hole 1a and the smaller-diameter electrode holding hole 1b which are defined respectively in the opposite ends of the bulb the bulb may be of a cylindrical shape with its both ends being simply open or may be a curved bulb.

In the fabrication process according to the first embodiment, each of the mixed slurries is coated and dried in forming the laminated body 20 around the support shaft 4 of tungsten which supports the main electrode 3. However, green sheets may be produced from the respective mixed slurries, and successively wound around the support shaft 4 in a descending order of volume ratios of tungsten. In this case, it is preferable to stack the green sheets such that the joined surfaces of the green sheets are alternately staggered 180° around the support shaft.

In joining the closures 2a and the bulb to each other in solid phase, the contacting surfaces are locally heated. However, they may be heated in the vicinity of the support shaft 4. Even when they are heated in the vicinity of the support shaft 4, since the applied thermal energy is transmitted to the outermost layers of the closures 2a, the closures 2a and the bulb can be joined to each other in solid phase. The closures 2a may be fired while the degreased closures 2a are being assembled in the bulb.

The gradient of the volume ratios of alumina and tungsten in the mixed slurries is not limited to the values indicated in the above embodiments, but may be of any of various other values.

The closure may be made of a gradient function material whose compositional proportions vary linearly from the core toward the bulb.

The first embodiment described above offers the following advantages:

In the light-emitting bulb assemblies according to the first embodiment, the closure joined in solid phase to the opening of the bulb which is made of light-transmissive ceramic comprises a multilayer laminated body, and the distribution of coefficients of thermal expansion from the innermost layer near the central conductive core toward the outermost layer near the bulb is a gradient distribution ranging from the coefficient of thermal expansion of the conductive core toward the coefficient of thermal expansion of the bulb based on the gradient of composition ratios of the layers.

Therefore, the compositions of the layers may be of a gradient pattern, and the layers, and the closure and the bulb may be firmly hermetically joined to each other in solid phase.

Based on the gradient distribution of the coefficients of thermal expansion, the concentration of thermal stresses produced upon energization of the bulb assembly can be reduced to avoid cracks in the solid-phase joints. As a result, the materials sealed in the bulb assembly are prevented from leaking out, so that the bulb assembly is capable of highly reliable light emission and has a prolonged service life.

The light-emitting bulb assemblies according to the above embodiment have a bulb made of light-transmissive alumina having an average particle diameter of 1 µm or less and a maximum particle diameter of 2 µm or less. Consequently, the mechanical strength of the light-emitting bulb assemblies ranging from normal temperature to a discharging temperature is higher than that of the conventional light-emitting bulb assemblies. Therefore, the wall thickness of the light-emitting bulb assemblies can be reduced to 0.2 mm or smaller, which is about 1/3 of that of the conventional light-emitting bulb assemblies.

Since almost no grain boundary phase such as a spinel phase is formed and crystallite boundaries in crystal grains which are responsible for diffusing light are reduced based on the small particle diameter, diffusion of light while the light is passing through the wall of the bulb is suppressed, thus providing high linear transmittance with respect to light (visible light) having a wavelength ranging from 380 to 760 nm. Consequently, the amount of light transmitted from a high-luminance discharge light-emitting bulb assembly is made greater than that from a conventional light-emitting bulb assembly, and hence the luminance of a high-pressure discharge lamp which employs a high-luminance discharge light-emitting bulb assembly is increased. That is, the amount of light transmitted from a high-luminance discharge light-emitting bulb assembly at the time light is applied to the high-luminance discharge light-emitting bulb assembly is made substantially equal to the amount of light applied to the high-luminance discharge light-emitting bulb assembly by suppressing diffusion of light. The luminance can further be increased by thinning out the wall of the bulb.

Inasmuch as the closure is fired and fabricated of highly pure alumina, the mechanical strength of the closure is increased, and the durability of the light-emitting bulb assembly as a whole is also increased.

According to the processes of manufacturing the light-emitting bulb assemblies according to the first embodiment, a plurality of suspensions with different volume ratios are prepared, a laminated closure having a gradient distribution of coefficients of thermal expansion is fabricated using the prepared suspensions, and the closure and a bulb are firmly hermetically joined in solid phase to each other. Thus, a light-emitting bulb assembly which is highly reliable and has a long service life can easily be manufactured. A laminated closure having a gradient distribution of coefficients of thermal expansion may separately be fired and fabricated, and joined in solid phase to a bulb.

According to the process of manufacturing the light-emitting bulb assembly according to the first embodiment, thin layers are successively stacked in an order of volume ratios of a conductive component (or a core) by repeating a simple process of pouring a suspension into a porous mold assembly, causing the solvent to penetrate into the mold assembly, and discharging the excessive suspension, for thereby easily producing an unfired laminated body which is a precursor of a laminated closure having a gradient distribution of coefficients of thermal expansion. The thicknesses of the thin layers can be uniformized for reliably maintaining composition distributions in the layers and a gradient distribution of coefficients of thermal expansion.

The central layer capable of being connected to an external source is formed of the conductive component within the innermost layer of the closure, and a given voltage can be applied without fail through the central layer to the main electrode.

A sealing structure of a light-emitting bulb assembly according to a second embodiment of the present invention and a method of manufacturing such a sealing structure will be described below with reference to Figs. 16 through 19.

Fig. 16 is a cross-sectional view of a light-emitting bulb assembly, particularly showing in detail a sealing structure of a bulb incorporated in an outer tube of a metal vapor discharge lamp.

A bulb 301 has openings 302 defined respectively in its opposite ends. End caps 303 as closures are integrally attached to the respective open ends 302, and electrode rods 304 as cores of the closures extend through and are held by the end caps 303, respectively.

The bulb 301 is made of light-transmissive polycrystalline alumina, and the electrode rods 304 are made of a tungsten-base material of W/Th or the like which is highly resistant to light-emitting substances. Each of the electrode rods 304 has an externally threaded portion 305 threaded in the corresponding end cap 303 and a flange 306 held against an outer end surface of the end cap 303. The flange 306 has an outer surface sealed by a sealant 307 such as of platinum solder or glass, and one of the electrode rods 304 has a hole 308 defined therein for introducing amalgam.

Each of the end caps 303 is of a multilayer structure as with the above embodiments. More specifically, each of the end caps 303 is composed of a plurality of layers 303₁, 303₂, ···, 303ₙ arranged along the axial direction of the bulb 1. The layer 303₁ (the bulb-side region layer) joined to the open end 302 of the bulb 301 has a coefficient of thermal expansion which is substantially the same as that of the light-transmissive alumina of which the bulb 301 is made. The outermost layer 303ₙ (the core-side region layer) has an internally threaded surface 309 in which the externally threaded portion 305 of the electrode rod 304 is threaded. The outermost layer 303ₙ has a coefficient of thermal expansion which is substantially the same as that of the electrode rod 304. The compositional proportions of the intermediate layers 303₂, ···, 303ₙ₋₁ (intermediate region layers) interposed between the layers 303₁, 303ₙ are adjusted such that the intermediate layers 303₂, ···, 303ₙ₋₁ have respective coefficients of thermal expansion varying gradually from that of the innermost layer 303₁ toward that of the outermost layer 303ₙ.

The thicknesses of the respective layers increase progressively from the innermost layer 303₁ toward the outermost layer 303ₙ. This is effective to reducing stresses that are developed when the layers are thermally expanded.

A tapered gap 310 is defined between the electrode rod 304 and the layers 303₁, ···, 303ₙ₋₁ except the outermost layer 303ₙ. The tapered gap 310 prevents the layers 303₁, ···, 303ₙ₋₁ from contacting the electrode rod 304 when the lamp is assembled.

A process of manufacturing the light-emitting bulb assembly of the above structure for a metal vapor discharge lamp will be described below with reference to Figs. 17 and 18(a) through 18 (e).

First, slips for fabricating the end caps 303 are prepared. To prepare such slips, as many containers C₁ ··· Cₙ as the number (n) of layers of each of the end caps 303 are employed as shown in Fig. 17. Material powders are weighed for obtaining desired coefficients of thermal expansion, and distilled water, a commercially available dispersing agent and a binder are added to the weighed material powders. They are then uniformly mixed for 24 hours by a ball mill, thereby producing slips S₁ ··· Sₙ respectively in the containers C₁ ··· Cₙ.

Table 7, given below, shows compositional proportions of material powders of respective slips for an end cap 303 which is composed of a total of eleven layers. In Table 7, the compositional proportions are represented by weight %, and the slip No. corresponds to the number of a layer of the end cap 303.

**Table 7**

| Slip No. | Al₂O₃ | W | Ni |
|---|---|---|---|
| 1 | 100 | 0 | 0 |
| 2 | 90 | 9 | 1 |
| 3 | 80 | 18 | 2 |
| 4 | 70 | 27 | 3 |
| 5 | 60 | 36 | 4 |
| 6 | 50 | 45 | 5 |
| 7 | 40 | 54 | 6 |
| 8 | 30 | 63 | 7 |
| 9 | 20 | 72 | 8 |
| 10 | 10 | 81 | 9 |
| 11 | 0 | 90 | 10 |

Then, as shown in Fig. 18(a), a tubular mold 312 is set on a porous plate or plaster board 311, and the slips S₁ ··· Sₙ prepared as described above are successively poured into the mold 312, thereby molding a laminated body. When each of the slips S₁ ··· Sₙ is to be poured, it is poured after the previously poured slip has lost its water content to a certain extent so that they will not be mixed with each other and the solvent of the previously poured slip will penetrate into the board 311.

As shown in Fig. 18(b), a mold bar 313 may be set either before or after the slips are poured. When the laminated body is partly dried, the laminated body is removed from the mold 312. The removed laminated body serves as an end cap 303 with a tapered through hole 314 defined therein as shown in Fig. 18(c). The through hole 314 may be of a stepped shape as shown in Fig. 18(d).

A bulb 301 molded of a pure alumina slip is prepared, and the end cap 303 which is made wet is joined to an end of the bulb 301 as shown in Fig. 18(e), after which the bulb 301 and the end cap 303 are dried. At this time, the bulb 301 and the end cap 303 are unfired, and the bulb 301 is not light-transmissive.

Then, the bulb 301 and the end cap 303 are degreased at 600°C for 5 hours in a moisture-containing hydrogen reducing atmosphere, and then fired at 1300°C for 5 hours in a dry hydrogen reducing atmosphere. Thereafter, the produced fired body is subjected to HIP in an argon atmosphere, and then annealed at 1150°C in a dry hydrogen reducing atmosphere, thereby producing an integral body of the light-transmissive bulb 301 and the end cap 303.

The hole 314 defined in the end cap 303 is tapped to produce an internally threaded surface 309, and then an electrode rod 304 is inserted and an externally threaded portion 305 of the electrode rod 304 is threaded in the internally threaded surface 309. Finally, the electrode rod 304 is fixed and sealed by a platinum solder 307, and an amalgam introduced into the bulb 301 through a hole 308 defined in the electrode rod 304 by a jig in the form of a platinum pipe. In this manner, the lamp is completed.

While the bulb and the end cap are simultaneously fired in the illustrated embodiment, they may be separately fired and then joined to each other. According to such a modification, the bulb of alumina may be degreased and fired in the atmosphere, then subjected to HIP, and thereafter annealed into a light-transmissive bulb of alumina. The end cap which is fired in the same manner as described above may not be subjected to HIP and annealed. The bulb and the end cap may be joined to each other by laser heating in vacuum or at 2000°C or higher, or glass having the same coefficient of thermal expansion as alumina. The glass should preferably be melted high-melting-point glass of a high softening point of 900°C or higher.

The end cap may be formed by a doctor blade process or an injection molding process as well as the slip casting process.

In the doctor blade process, prepared slurries are formed into tapes of desired thicknesses, and the tapes are integrally joined together into an end cap having a gradient function by thermal compression. The same slurries may be used to cast the bulb or poured into a mold and then solidified into the bulb.

In the injection molding process, sheets of desired thicknesses are formed and bonded together with heat, thus producing an end cap which will be joined to a previously molded bulb by thermal compression.

According to the second embodiment, each of the end caps which seal the open ends of a metal vapor discharge lamp is of a multilayer structure, and the coefficients of thermal expansion of the layers vary gradually from the open end of the bulb toward the core which holds an electrode, so that the end caps have a gradient function. Consequently, the end caps are effective to prevent damage due to different thermal expansions and leakage of the metal vapor sealed in the bulb.

Fig. 19 shows a modification of the second embodiment. According to the modification, a bulb 301' differs from the bulb 301 shown in Fig. 16 in that the opposite ends of the bulb are not fully open, but have respective end surfaces 301a. The end surfaces 301a have respective small openings as large as a larger-diameter portion of the tapered through hole 314 for allowing the electrode rods 304 to be inserted therethrough into the bulb.

Light-emitting bulb assemblies according to third embodiment will be described below with reference to Figs. 24 through 27(a) and 27(b).

In the third embodiment, a tubular bulb 521 is made of light-transmissive polycrystalline alumina having a high purity of 99.99 % = 4N, and electrode sealing members 523 of a laminated structure made of alumina of low purity are disposed on respective opposite ends 522 of the bulb 521. Electrode rods 524 as cores are inserted respectively in the electrode sealing members 523. Caps 525 of alumina through which the electrode rods 524 extend are disposed outside of the electrode sealing members 523, and the electrode sealing members 523, the electrode rods 524, and the caps 525 are sealed by sealing glass 526.

The electrode sealing members 523 is made of an alumina material which has a lower purity (e.g., 99 ∼ 97 %) than the bulb 521 which serves as a light-emitting portion. Each of the electrode sealing members 523 is of a laminated structure including a first layer 523a, a second layer 523b, and a third layer 523c (the laminated structure may include four or more layers) arranged along the axial direction of the bulb 521 or the electrode rods 524. The first layer 523a, the second layer 523b, and the third layer 523c are progressively thicker in the direction from the first layer 523a toward the third layer 523c. As a result, the third layer 523c and the second layer 523b have a greater area held against the electrode rods 524 than the first layer 523a. The caps 525 are made of alumina having the same purity as that of the third layer 523c.

The caps 525 may be dispensed with as required.

A process of manufacturing the above ceramic light-emitting bulb assembly will be described below with reference to Figs. 25 through 27(a) and 27(b).

First, a fine powder of alumina having a high purity of 4N or more for producing light-transmissive alumina, and a fine powder of alumina having a lower purity (93 % in this embodiment) are prepared. To the powders which have been weighed, there are added predetermined amounts of distilled water, a commercially available dispersing agent, and a binder. The materials are then mixed for 24 hours by a ball mill, thereby producing, as shown in Fig. 25, an alumina slip S₅₁ having a high purity (4N) is prepared in a container C₅₁, an alumina slip S₅₂ having a purity of 97 % in a container C₅₂, an alumina slip S₅₃ having a purity of 95 % in a container C₅₃, and an alumina slip S₅₄ having a purity of 93 % in a container C₅₄.

Thereafter, as shown in Fig. 27(a), a tubular mold 532 having a size matching the outside diameter of a bulb is set on a porous mold assembly or plaster mold assembly 531, and a mold bar 533 is vertically placed centrally in the mold 532. Then, the alumina slip S₅₄ having a purity of 93 %, the alumina slip S₅₃ having a purity of 95 %, the alumina slip S₅₂ having a purity of 97 %, and the alumina slip S₅₁ having a high purity are successively poured into a space defined by the mold 532 and the mold bar 533, thereby molding a laminated body. When each of the alumina slips is to be poured, it is poured after the previously poured slip has lost its water content to a certain extent so that they will not be mixed with each other.

A pipe 534 shown in Fig. 26 which will serve as the bulb 521 is formed of the highly pure alumina slip S₅₁. The pipe 534 is then inserted into the mold 532 while the highly pure alumina slip S₅₁ for producing an end 522a of the bulb 521 is not being dried, and integrally joined to the laminated body, thereby producing a molded body as shown in Fig. 27(b). Thereafter, as with the above embodiment, the molded body is fired, machined, and assembled.

With the present invention, as described above, electrode sealing members made of an alumina material having a lower purity than a light-emitting portion are disposed on respective opposite ends of a bulb, and a glass solder or sealing glass is held in contact with the electrode sealing members to keep them out of contact with the bulb. Therefore, the sealing capability is made highly reliable for allowing the lamp to have an increased service life.

As with the above embodiment, since the composition of the electrode sealing members is of a gradient nature, the sealing capability of the sealing regions is further increased.

A sealing structure of a light-emitting bulb assembly for a metal vapor discharge lamp according to a fourth embodiment of the present invention and a method of manufacturing such a sealing structure will be described below with reference to Figs. 28 through 30(a) ∼ 30(d).

Fig. 28 shows a bulb 601 made of light-transmissive polycrystalline alumina to be incorporated in an outer tube of a metal vapor discharge lamp. Caps 604 of alumina as closures are fitted in respective end openings 602 of the bulb 601 through sealing glass 603.

Each of the caps 604 comprises a high-purity alumina portion 604a, a gradient-composition portion 604b, and a low-purity alumina portion 604c. The high-purity alumina portion 604a as a bulb-side region is made of Al₂O₃ having a purity of 99.99 % and exposed to the interior of the bulb 601. The low-purity alumina portion 604c as a core-side region is made of Al₂O₃ having a purity of 93.0 % and exposed to the exterior of the bulb 601. The gradient-composition portion 604b as an intermediate region has a section held against the high-purity alumina portion 604a and having a purity of 99.99 %, is progressively lower in purity toward the low-purity alumina portion 604c, and has a section held against the low-purity alumina portion 604c and having a purity of 93.0 %. The gradient-composition portion 604b with such a continuous gradient composition has a greatly increased peeling strength. The low-purity alumina portion 604c has a greater width along the axial direction of the bulb than the width of the high-purity alumina portion 604a.

As shown in Fig. 29(d), each of the caps 604 has axial holes 605, 606 defined therein. An internal electrode rod 607 is press in the hole 605, and an external electrode rod (lead) 608 is pressed in the hole 606. The holes 605, 606 are such diameters which will be about 200 µm larger than electrode rods 607, 608 after being fired. This prevents the caps from being obstructed and cracked by the electrodes when fired.

The low-purity alumina portion 604c has a radial hole 609 defined from its side toward the inside thereof in communication with the axial hole 605. A conductive film 610 of tungsten (W) or the like is disposed in the radial hole 609 and on the outer surface of the low-purity alumina portion 604c. The conductive film 610 serves to provide a good electric connection between the internal electrode rod 607 and the external electrode rod 608. The conductive film 610 may be made of Nb, Ta, Mo, Ni, or the like.

A process of manufacturing each of the caps 604 will be described below with reference to Figs. 29(a) through 29(e). First, as shown in Fig 29(a), 100 g of Al₂O₃ of a high purity (99.99 %), 100 g of Al₂O₃ of a low purity (93.0 %), 50 g of water, and a deflocculant are mixed for 24 hours by a ball mill, thereby producing a slip S₆₁ of Al₂O₃ of a high purity and a slip S₆₂ of Al₂O₃ of a low purity.

Then, as shown in Fig. 29(b), the slips S₆₁, S₆₂ are mixed with each other to produce a plurality of slips S₆₃ having purities ranging between 99.99 % and 93.0 %. Thereafter, as shown in Fig. 29(c), the slips are successively poured, from the highly pure slip S₆₁, into a mold 615 set on a porous body or a plaster body 614, producing a molded body 616 prior to being fired by way of one-sided deposition.

The molded body 616 is then temporarily fired at 1100°C for 2 hours, so that the molded body 616 has a hardness that allows the molded body 616 to be handled. Thereafter, the molded body 616 is machined to form axial holes 605, 606 and a radial hole 609, as shown in Fig. 19(d), and shaped into a cap. A conductive paste 610 is then introduced into the radial hole 609 and applied to the outer surface of the low-purity alumina portion 604c. With the internal electrode rod 607 and the external electrode rod 608 being inserted, the assembly is fired at 1570°C for 3 hours in an atmosphere of N₂ and H₂ (N₂ : H₂ = 80 : 20), thereby producing a cap 604 as shown in Fig. 29(e). The cap 604 is inserted in one of the openings 602 of the bulb 601, and sealed by glass 603 or an alloy of a low melting point.

Figs. 30(a) through 30(d) show a modification of the process of manufacturing the light-emitting body according to the fourth embodiment. According to the modified process, as shown in Fig. 30(a), using two porous bodies or plaster bodies 614a, 614b and two molds 615a, 615b, a molded body 616a serving as a high-purity alumina portion and a gradient-composition portion, and a molded body 616b serving as a low-purity alumina portion are produced as shown in Fig. 30(b).

Then, as shown in Fig. 30(c), the surface of the molded body 616b is coated with a conductive paste, and the molded body 616a is bonded integrally to the molded body 616b by the conductive paste. Subsequently, an internal electrode rod 607 and an external electrode rod 608 are inserted, and the assembly is fired into a cap 604 as shown in Fig. 30(d). Since the conductive paste which interconnects the molded bodies 616a, 616b provides an electric connection between the internal electrode rod 607 and the external electrode rod 608, the radial hole 609 as shown in Fig. 29(d) is not required.

According to the fourth embodiment as described above, each of caps which close respective openings of a light-emitting bulb assembly for a metal vapor discharge lamp and support internal and external electrodes separately from each other is composed of a high-purity alumina portion exposed to the interior of the bulb assembly, a low-purity alumina portion exposed to the exterior of the bulb assembly, and a gradient-composition portion interconnecting the high-purity alumina portion and the low-purity alumina portion, and a conductive film which provides an electric connection between the internal and external electrodes is disposed on the surface of the low-purity alumina portion. The conductive film has a peeling strength increased to 10 kg/cm² from a conventional value ranging from 1 to 4 kg/cm².

Since the high-purity alumina portion is exposed to the interior of the bulb assembly, the lamp characteristics are prevented from being degraded due to a corrosive component such as Na. As no conductive film is disposed on the high-purity alumina portion and the gradient-composition portion, no back arcs are produced. Metals such as Nb, Ta, Mo, Ti, and so on may also be used as the conductive film (metallized film).

### Industrial Applicability

A sealing structure for a light-emitting bulb assembly allows a discharge light-emitting bulb assembly to be highly reliable and have a long service life. The light-emitting bulb assembly can be used in a metal-vapor discharge lamp such as a mercury-vapor lamp, a metal halide lamp, or a sodium-vapor lamp, or a high-intensity discharge lamp.

## Claims

1. A light-emitting bulb having a sealing structure, which includes a closure (303), having a core (304) which serves as an electrode, for sealing an open end (302) of the bulb, said closure including a bulb-side region (303₁) disposed adjacent to the open end of said bulb and made of a compositional ingredient having a coefficient of thermal expansion which is substantially'the same as that of the bulb, a core-side region (303ₙ) disposed adjacent to said core and made of a compositional ingredient having a coefficient of thermal expansion which is substantially the same as that of the core, and an intermediate region (303₂ - 303ₙ₋₁) disposed between said bulb-side region and said core-side region and made of a compositional ingredient having compositional proportions adjusted such that the coefficient of thermal expansion thereof varies gradually from the coefficient of thermal expansion of said bulb-side region towards the coefficient of thermal expansion of said core-side region; wherein said bulb-side region and said core-side region comprise a bulb-side region layer and a core-side region layer, respectively, which are independent of each other, and wherein said intermediate region comprises at least one layer whose coefficient of thermal expansion varies gradually from said bulb-side region towards said core-side region; and wherein said at least one layer of the bulb-side region, the intermediate region and said core-side region layer are successively arranged in an axial direction of said bulb.

2. A bulb according to claim 1, wherein the layers of said closure are progressively thicker from said bulb-side region layer towards said core-side region layer.

3. A bulb according to claim 1, wherein a metal vapor is sealed in said light-emitting bulb assembly.

4. A bulb according to claim 1, wherein said closure is made of a material whose compositional proportions vary linearly at least from said bulb-side region through said intermediate region to said core-side region.

5. A bulb according to claim 1, wherein said bulb is made of light-transmissive ceramic.

6. A bulb according to claim 5, wherein said bulb is made of light-transmissive alumina.

7. A bulb according to claim 6, wherein said light-transmissive alumina of the bulb comprises a fired fine powder of alumina having a high purity of at least 99.99 mol %, said light-transmissive alumina having crystal grains having an average particle diameter of at most 1 µm and a maximum particle diameter of at most 2 µm.

8. A bulb according to claim 7, wherein the compositional ingredient of said bulb-side region includes alumina having a high purity, the compositional ingredient of said core-side region includes alumina having a low purity, and the compositional ingredient of said intermediate region includes alumina having a graded intermediate purity.

9. A bulb according to claim 5, wherein said bulb-side region includes at least 80% by volume of said light-transmissive ceramic, and said core-side region includes at least 50% by volume of a compositional ingredient of said core.

10. A bulb according to claim 9, wherein the compositional ingredient of said intermediate region includes light-transmissive ceramic having a volume ratio which is progressively closer to the volume ratio of the light-transmissive ceramic of said bulb-side region in a direction toward said bulb-side region, and also includes the compositional ingredient of said core having a volume ratio which is progressively closer to the volume ratio of the compositional ingredient of said core in said core-side region layer in a direction toward said core-side region layer.

11. A bulb according to claim 10, wherein said light-transmissive ceramic includes alumina having a high purity, and said compositional ingredient of said core includes tungsten.

12. A bulb according to claim 1, wherein said closure has an electrode rod as said core which extends through said closure and supports said electrode so as to position the electrode in the light-emitting bulb assembly, and wherein said bulb-side region layer is joined to said open end of the bulb.

13. A bulb according to claim 12, wherein the layers of said closure are progressively thicker from said bulb-side region layer toward said core-side region layer.

14. A bulb according to claim 12, wherein a gap is disposed between said bulb-side region layer, said at least one layer of the intermediate region, and said electrode rod.

15. A bulb according to claim 13, wherein said core-side region layer and said at least one layer of the intermediate region have a greater area disposed adjacent to said electrode rod than said bulb-side region layer, and wherein said bulb-side region layer, said at least one layer of the intermediate region, and said core-side region layer are disposed adjacent said electrode rod through a glass solder interposed therebetween.

16. A bulb according to claim 1, wherein said core is positioned substantially centrally in said closure, and said bulb-side region layer, said at least one layer of the intermediate region, and said core-side region layer are stacked in an axial direction of said core, said bulb-side region layer being exposed to an interior of said bulb and disposed adjacent to said bulb.

17. A bulb according to claim 16, wherein said core-side region layer has a greater area disposed adjacent to said core than said at least one layer of the intermediate region and said bulb-side region layer.

18. A bulb according to claim 17, wherein said core has an internal electrode rod extending from said core-side region layer to said bulb-side region layer and projecting into said bulb and having an electrode on a distal end thereof, and an external electrode rod projecting from said core-side region layer out of said bulb.

19. A bulb according to claim 18, wherein a conductive layer is disposed on an outer surface of said core-side region layer and provides an electric connection between said internal electrode rod and said external electrode rod.

20. A bulb according to claim 19, wherein said core-side region layer has a through hole defined therein from a side of said core-side region layer to said internal electrode rod, said conductive layer being disposed in said through hole and providing said electric connection between said internal electrode rod and said external electrode rod.

21. A bulb according to claim 19, wherein said closure is joined to said open end of said bulb through sealing glass.

22. A method of manufacturing a light-emitting bulb according to claim 1 comprising the steps of:
(a) preparing, from a fine powder of a light-transmissive bulb ingredient and a fine powder of a core ingredient, a bulb ingredient suspension in which the light-transmissive bulb ingredient is greater than the core ingredient, a core ingredient suspension in which the core ingredient is greater than the light-transmissive bulb ingredient, and at least one intermediate suspension in which the light-transmissive bulb ingredient and the core ingredient have compositional proportions lying between those of said bulb ingredient suspension and said core ingredient suspension;
(b) forming an unfired laminated body composed of an unfired bulb-side region layer to be disposed adjacent to said light-transmissive bulb and formed from said bulb ingredient suspension, an unfired core-side region layer to be disposed adjacent to said core and formed from said core ingredient suspension, and at least one unfired intermediate region layer disposed between said unfired bulb-side region layer and said unfired core-side region layer and formed from said at least one intermediate suspension; and
(c) firing said unfired laminated body;
wherein said step (b) comprises the step of:
(g) successively pouring said core ingredient suspension, said at least one intermediate suspension, and said bulb ingredient suspension into a mold which comprises a tubular body vertically mounted on a porous plate to form said core-side region layer, said intermediate region layer, and said bulb-side region layer, respectively, thereby forming said unfired laminated body.

23. A method according to claim 22, wherein said step (g) comprises the step of:
vertically placing a tapered mold bar centrally in said mold to define a through hole in said closure for said core to extend therethrough.

24. A method according to claim 22, wherein said step (c) comprises the, steps of:
molding an unfired bulb from the fine powder of the light-transmissive bulb ingredient, and joining said unfired laminated body to an open end of said unfired bulb.

25. A method according to claim 22, wherein said step (a) comprises the steps of:
preparing a purely bulb suspension from the fine powder of said light-transmissive bulb ingredient, and forming an unfired bulb tubular body to be formed into said light-transmissive bulb from said purely bulb suspension;
wherein said step (g) comprises the step of:
after said unfired laminated body composed of said core-side region layer, said intermediate region layer, and said bulb-side region layer has been formed, integrally placing said unfired bulb tubular body on said bulb-side region layer of said unfired laminated body; and
wherein said step (c) comprises the step of:
firing said unfired laminated body including said unfired bulb tubular body.

## Patentansprüche

1. Lichtemittierender Kolben mit Abdichtstruktur, die einen Verschluss (303) mit einem als Elektrode dienenden Kern (304) enthält, um ein offenes Ende (302) des Kolbens abzudichten, wobei der Verschluss umfasst: einen kolbenseitigen Bereich (303₁), der benachbart dem offenen Ende des Kolbens angeordnet und aus einem Zusammensetzungsbestandteil hergestellt ist, der einen thermischen Ausdehnungskoeffizienten hat, der im Wesentlichen der gleiche ist wie jener des Kolbens, einen kernseitigen Bereich (303ₙ), der benachbart dem Kern angeordnet und aus einem Zusammensetzungsbestandteil hergestellt ist, der einen thermischen Ausdehnungskoeffizienten hat, der im Wesentlichen der gleiche ist wie jener des Kerns, sowie einen Zwischenbereich (303₂ - 303ₙ₋₁), der zwischen dem kolbenseitigen Bereich und dem kernseitigen Bereich angeordnet und aus einem Zusammensetzungsbestandteil hergestellt ist, der derart eingestellte Zusammensetzungseigenschaften hat, dass sich sein thermischer Ausdehnungskoeffizient graduell von dem thermischen Ausdehnungskoeffizienten des kolbenseitigen Bereichs zu dem thermischen Ausdehnungskoeffizienten des kernseitigen Bereichs hin ändert; worin der kolbenseitige Bereich und der kernseitige Bereich eine kolbenseitige Bereichsschicht bzw. eine kernseitige Bereichsschicht aufweist, die voneinander unabhängig sind, und worin der Zwischenbereich zumindest eine Schicht aufweist, deren thermischer Ausdehnungskoeffizient sich graduell von dem kolbenseitigen Bereich zum kernseitigen Bereich hin ändert; und worin die zumindest eine Schicht des kolbenseitigen Bereichs, der Zwischenbereich und die kernseitige Bereichsschicht in axialer Richtung des Kolbens aufeinanderfolgend angeordnet sind.

2. Kolben nach Anspruch 1, worin die Schichten des Verschlusses von der kolbenseitigen Bereichsschicht zur kernseitigen Bereichsschicht hin progressiv dicker sind.

3. Kolben nach Anspruch 1, worin in der lichtemittierenden Kolbenanordnung Metalldampf eingeschlossen ist.

4. Kolben nach Anspruch 1, worin der Verschluss aus einem Material hergestellt ist, dessen Zusammensetzungsproportionen sich linear zumindest von dem kolbenseitigen Bereich durch den Zwischenbereich zu dem kernseitigen Bereich hin ändern.

5. Kolben nach Anspruch 1, worin der Kolben aus lichtdurchlässiger Keramik hergestellt ist.

6. Kolben nach Anspruch 5, worin der Kolben aus lichtdurchlässigem Aluminiumoxid hergestellt ist.

7. Kolben nach Anspruch 6, worin das lichtdurchlässige Aluminiumoxid des Kolbens ein gebranntes feines Aluminiumoxidpulver mit einer hohen Reinheit von zumindest 99,99 Mol-% aufweist, wobei das lichtdurchlässige Aluminiumoxid Kristallkörner mit einem durchschnittlichen Partikeldurchmesser von höchstens 1 µm und einem maximalen Partikeldurchmesser von höchstens 2 µm aufweist.

8. Kolben nach Anspruch 7, worin der Zusammensetzungsbestandteil des kolbenseitigen Bereichs Aluminiumoxid mit hoher Reinheit enthält, der Zusammensetzungsbestandteil des kernseitigen Bereichs Aluminiumoxid mit niedriger Reinheit enthält und der Zusammensetzungsbestandteil des Zwischenbereichs Aluminiumoxid mit mittelmäßiger Reinheit enthält.

9. Kolben nach Anspruch 5, worin der kolbenseitige Bereich zumindest 80 Volumen-% der lichtdurchlässigen Keramik enthält und der kernseitige Bereich zumindest 50 Volumen-% eines Zusammensetzungsbestandteils des Kerns enthält.

10. Kolben nach Anspruch 9, worin der Zusammensetzungsbestandteil des Zwischenbereichs lichtdurchlässige Keramik mit einem Volumenverhältnis enthält, das sich in Richtung zu dem kolbenseitigen Bereich hin dem Volumenverhältnis der lichtdurchlässigen Keramik des kolbenseitigen Bereichs progressiv annähert, und ferner den Zusammensetzungsbestandteil des Kerns mit einem Volumenverhältnis enthält, das sich in Richtung zu der kernseitigen Bereichsschicht hin dem Volumenverhältnis des Zusammensetzungsbestandteils des Kerns in der kernseitigen Bereichsschicht progressiv annähert.

11. Kolben nach Anspruch 10, worin die lichtdurchlässige Keramik Aluminiumoxid mit hoher Reinheit enthält und der Zusammensetzungsbestandteil des Kerns Wolfram enthält.

12. Kolben nach Anspruch 1, worin der Verschluss als den Kern eine Elektrodenstange aufweist, die sich durch den Verschluss erstreckt und die Elektrode hält, um die Elektrode in der lichtemittierenden Kolbenanordnung zu positionieren, und worin die kolbenseitige Bereichsschicht mit dem offenen Ende des Kolbens verbunden ist.

13. Kolben nach Anspruch 12, worin die Schichten des Verschlusses von der kolbenseitigen Bereichsschicht zu der kernseitigen Bereichsschicht hin progressiv dicker sind.

14. Kolben nach Anspruch 12, worin zwischen der kolbenseitigen Bereichsschicht, der zumindest einen Schicht des Zwischenbereichs und der Elektrodenstange ein Spalt angeordnet ist.

15. Kolben nach Anspruch 13, worin die kernseitige Bereichsschicht und die zumindest eine Schicht des Zwischenbereichs eine der Elektrodenstange benachbart angeordnete größere Fläche haben als die kolbenseitige Bereichsschicht, und worin die kolbenseitige Bereichsschicht, die zumindest eine Schicht des Zwischenbereichs und die kernseitige Bereichsschicht benachbart der Elektrodenstange durch eine dazwischen befindliche Glasverschmelzung angeordnet sind.

16. Kolben nach Anspruch 1, worin der Kern im Wesentlichen in der Mitte des Verschlusses angeordnet ist, und die kolbenseitige Bereichsschicht, die zumindest eine Schicht des Zwischenbereichs und die kernseitige Bereichsschicht in axialer Richtung des Kerns gestapelt sind, wobei die kolbenseitige Bereichsschicht zum Inneren des Kolbens frei liegt und dem Kolben benachbart angeordnet ist.

17. Kolben nach Anspruch 16, worin die kernseitige Bereichsschicht eine dem Kern benachbart angeordnete größere Fläche hat als die zumindest eine Schicht des Zwischenbereichs und die kolbenseitige Bereichsschicht

18. Kolben nach Anspruch 17, worin der Kern eine innere Elektrodenstange aufweist, die sich von der kernseitigen Bereichsschicht zu der kolbenseitigen Bereichsschicht erstreckt und in den Kolben vorsteht und an ihrem distalen Ende eine Elektrode aufweist, sowie eine äußere Elektrodenstange, die von der kernseitigen Bereichsschicht aus dem Kolben vorsteht.

19. Kolben nach Anspruch 18, worin auf einer Außenfläche der kernseitigen Bereiehsschicht eine leitfähige Schicht angeordnet ist und eine elektrische Verbindung zwischen der inneren Elektrodenstange und der äußeren Elektrodenstange herstellt.

20. Kolben nach Anspruch 19, worin die kernseitige Bereichsschicht ein Durchgangsloch aufweist, das darin von einer Seite der kernseitigen Bereichsschicht zu der inneren Elektrodenstange hin definiert ist, wobei die leitfähige Schicht in dem Durchgangsloch angeordnet ist und die elektrische Verbindung zwischen der inneren Elektrodenstange und der äußeren Elektrodenstange herstellt.

21. Kolben nach Anspruch 19, worin der Verschluss mit dem offenen Ende des Kolbens durch Abdichtglas verbunden ist.

22. Verfahren der Herstellung eines lichtemittierenden Kolbens nach Anspruch 1, das die Schritte aufweist:
(a) Bereitstellen, aus einem feinen Pulver eines lichtdurchlässigen Kolbenbestandteils und einem feinen Pulver eines Kernbestandteils, einer Kolbenbestandteilsuspension, in der der lichtdurchlässige Kolbenbestandteil größer ist als der Kernbestandteil, einer Kernbestandteilsuspension, in der der Kernbestandteil größer ist als der lichtdurchlässige Kolbenbestandteil, und zumindest einer Zwischensuspension, in der der lichtdurchlässige Kolbenbestandteil und der Kernbestandteil Zusammensetzungsproportionen haben, die zwischen jenen der Kolbenbestandteilsuspension und der Kernbestandteilsuspension liegen;
(b) Bilden eines nicht-gebrannten geschichteten Körpers, der zusammengesetzt ist aus einer nicht gebrannnten kolbenseitigen Bereichsschicht, die benachbart dem lichtdurchlässigen Kolben anzuordnen und aus der Kolbenbestandteilsuspension gebildet ist, einer nicht gebrannten kernseitigen Bereichsschicht, die benachbart dem Kern anzuordnen und aus der Kernbestandteilsuspension gebildet ist, und zumindest einer nicht gebrannten Zwischenbereichsschicht, die zwischen der nicht gebrannten kolbenseitigen Bereichsschicht und der nicht gebrannten kernseitigen Bereichsschicht angeordnet und aus der zumindest einen Zwischensuspension gebildet ist; und
(c) Brennen des nicht gebrannten geschichteten Körpers;
worin der Schritt (b) den Schritt aufweist:
(g) aufeinanderfolgendes Gießen der Kernbestandteilsuspension, der zumindest einen Zwischensuspension und der Kolbenbestandteilsuspension in eine Form, die einen rohrförmigen Körper aufweist, der vertikal an einer porösen Platte angebracht ist, um jeweils die kernseitige Bereichsschicht, die Zwischenbereichsschicht und die kolbenseitige Bereichsschicht zu bilden, um hierdurch den nicht gebrannten geschichteten Körper zu bilden.

23. Verfahren nach Anspruch 22, worin der Schritt (g) den Schritt aufweist:
vertikales Anordnen einer verjüngten Formstange in der Mitte in der Form, um ein Durchgangsloch in dem Verschluss für den sich hierdurch erstreckenden Kern zu definieren.

24. Verfahren nach Anspruch 22, worin der Schritt (c) die Schritte aufweist:
Formen eines nicht gebrannten Kolbens aus dem feinen Pulver des lichtdurchlässigen Kolbenbestandteils und Verbinden des nicht gebrannten geschichteten Körpers mit einem offenen Ende des nicht gebrannten Kolbens.

25. Verfahren nach Anspruch 22, worin der Schritt (a) die Schritte aufweist:
Bereitstellen einer reinen Kolbensuspension aus dem feinen Pulver des lichtdurchlässigen Kolbenbestandteils und Bilden eines nicht gebrannten rohrförmigen Kolbenkörpers, der zu dem lichtdurchlässigen Kolben zu formen ist, aus der reinen
Kolbensuspension;
worin der Schritt (g) den Schritt aufweist:
nachdem der nicht gebrannte geschichtete Körper, der aus der kernseitigen Bereichsschicht, der Zwischenbereichsschicht und der kolbenseitigen Bereichsschicht zusammengesetzt ist, gebildet worden ist, integrales Anordnen des nicht gebrannten rohrförmigen Kolbenkörpers auf der kolbenseitigen Bereichsschicht des nicht gebrannten geschichteten Körpers; und
worin der Schritt (c) den Schritt aufweist:
Brennen des nicht gebrannten geschichteten Körpers, der den nicht gebrannten rohrförmigen Kolbenkörper enthält.

## Revendications

1. Ampoule à émission de lumière comportant une structure de scellement, laquelle inclut une enceinte (303), ayant un noyau (304) qui sert comme électrode, pour fermer une extrémité ouverte (302) de l'ampoule, ladite enceinte incluant une région côté ampoule (303₁) disposée adjacente à l'extrémité ouverte de ladite ampoule et constituée d'un ingrédient compositionnel présentant un coefficient de dilatation thermique qui est sensiblement le même que celui de l'ampoule, une région côté noyau (303ₙ) disposée adjacente audit noyau et constituée d'un ingrédient compositionnel présentant un coefficient de dilatation thermique qui est sensiblement que celui du noyau, une région intermédiaire (303₂ à 303ₙ₋₁) disposée entre ladite région côté ampoule et ladite région côté noyau et constituée d'un ingrédient compositionnel ayant des proportions compositionnelles ajustées de sorte que son coefficient de dilatation thermique varie progressivement à partir du coefficient de dilatation thermique de ladite région côté ampoule vers le coefficient de dilatation thermique de ladite région côté noyau ; dans laquelle ladite région côté ampoule et ladite région côté noyau comprennent une couche de région côté ampoule et une couche de région côté coeur, respectivement, qui sont mutuellement indépendantes, et dans laquelle ladite région intermédiaire comprend au moins une couche dont le coefficient de dilatation thermique varie progressivement à partir de ladite région côté ampoule vers ladite région côté noyau ; et dans lequel ladite au moins une couche de la région côté ampoule, de la région intermédiaire et ladite couche de la région côté noyau sont successivement disposées dans une direction axiale de ladite ampoule.

2. Ampoule selon la revendication 1, dans laquelle les couches de ladite enceinte sont progressivement plus épaisses en partant de ladite couche de région côté ampoule vers ladite couche de région côté noyau.

3. Ampoule selon la revendication 1, dans laquelle une vapeur métallique est enfermée dans ledit ensemble d'ampoules d'émission de lumière.

4. Ampoule selon la revendication 1, dans laquelle ladite enceinte est constituée d'un matériau dont les proportions compositionnelles varient linéairement au moins à partir de ladite région côté ampoule en passant par ladite région intermédiaire jusqu'à ladite région côté noyau.

5. Ampoule selon la revendication 1, dans laquelle ladite ampoule est constituée d'une céramique transmettant la lumière.

6. Ampoule selon la revendication 5, dans laquelle ladite ampoule est constituée d'une alumine transmettant la lumière.

7. Ampoule selon la revendication 6, dans laquelle ladite alumine transmettant la lumière de l'ampoule comprend une poudre fine cuite d'alumine ayant une pureté élevée d'au moins 99,99 mol %, ladite alumine transmettant la lumière ayant des grains de cristal présentant un diamètre particulaire moyen d'au plus 1 µm et un diamètre particulaire maximal d'au plus 2 µm.

8. Ampoule selon la revendication 7, dans laquelle l'ingrédient compositionnel de ladite région côté ampoule inclut de l'alumine ayant une pureté élevée, l'ingrédient compositionnel de ladite région côté noyau inclut de l'alumine ayant une faible pureté et l'ingrédient compositionnel de ladite région intermédiaire inclut une alumine ayant une pureté intermédiaire graduée.

9. Ampoule selon la revendication 5, dans laquelle ladite région côté ampoule inclut au moins 80 % en volume de ladite céramique transmettant la lumière, et ladite région côté noyau inclut au moins 50 % en volume d'un ingrédient compositionnel dudit noyau.

10. Ampoule selon la revendication 9, dans laquelle l'ingrédient compositionnel de ladite région intermédiaire inclut une céramique transmettant la lumière ayant un rapport de volume qui est progressivement plus proche du rapport en volume de la céramique transmettant la lumière de ladite région côté ampoule dans une direction vers ladite région côté ampoule, et inclut également l'ingrédient compositionnel dudit noyau ayant un rapport de volume qui est progressivement plus proche du rapport de volume de l'ingrédient compositionnel dudit noyau dans ladite couche de région côté noyau dans une direction vers ladite couche de région côté noyau.

11. Ampoule selon la revendication 10, dans laquelle ladite céramique transmettant la lumière inclut une alumine ayant une pureté élevée, et ledit ingrédient compositionnel dudit noyau inclut du tungstène.

12. Ampoule selon la revendication 1, dans laquelle ladite enceinte comporte une tige d'électrode comme ledit noyau qui s'étend à travers ladite enceinte et supporte ladite électrode de façon à positionner l'électrode dans l'ensemble d'ampoules émettant la lumière, et dans laquelle ladite couche de région côté ampoule est raccordée à ladite extrémité de l'ampoule.

13. Ampoule selon la revendication 12, dans laquelle les couches de ladite enceinte sont progressivement plus épaisses en partant de ladite couche de région côté ampoule vers ladite couche de région côté noyau.

14. Ampoule selon la revendication 12, dans laquelle un espace est ménagé entre ladite couche de région côté ampoule, ladite au moins une couche de la région intermédiaire et ladite tige d'électrode.

15. Ampoule selon la revendication 13, dans laquelle ladite couche de région côté noyau et ladite au moins une couche de la région intermédiaire ont une surface plus grande disposée adjacente à ladite tige d'électrode que ladite couche de région côté ampoule, et dans laquelle ladite couche de région côté ampoule, ladite au moins une couche de la région intermédiaire et ladite couche de région côté noyau sont disposées adjacentes à ladite tige d'électrode à travers une soudure en verre interposée entre celles-ci.

16. Ampoule selon la revendication 1, dans laquelle ledit noyau est positionné sensiblement au centre de ladite enceinte, et ladite couche de région côté ampoule, ladite au moins une couche de région intermédiaire et ladite couche de région côté noyau sont empilées dans une direction axiale dudit noyau, ladite couche de région côté ampoule étant exposée à l'intérieur de ladite ampoule et disposée adjacente à ladite ampoule.

17. Ampoule selon la revendication 16, dans laquelle ladite couche de région côté noyau comporte une surface plus grande disposée adjacente audit noyau que celle de ladite au moins une couche de la région intermédiaire et de ladite couche de région côté ampoule.

18. Ampoule selon la revendication 17, dans laquelle ledit noyau comporte une tige d'électrode interne s'étendant depuis ladite couche de région côté noyau vers ladite couche de région côté ampoule et dépassant dans ladite ampoule et ayant une électrode sur son extrémité distale, et une tige d'électrode externe dépassant depuis ladite couche de région côté noyau en dehors de ladite ampoule.

19. Ampoule selon la revendication 18, dans laquelle une couche conductrice est disposée sur une surface externe de ladite couche de région côté noyau et assure une connexion électrique entre ladite tige d'électrode interne et ladite tige d'électrode externe.

20. Ampoule selon la revendication 19, dans laquelle ladite couche de région côté noyau comporte un trou traversant défini dans celle-ci à partir d'un côté de ladite couche de région côté noyau jusqu'à ladite tige d'électrode interne, ladite couche conductrice étant disposée dans ledit trou traversant et assurant ladite connexion électrique entre ladite tige d'électrode interne et ladite tige d'électrode externe.

21. Ampoule selon la revendication 19, dans laquelle ladite enceinte est raccordée à ladite extrémité ouverte de ladite ampoule par l'intermédiaire d'un verre d'étanchéité.

22. Procédé de fabrication d'une ampoule à émission de lumière selon la revendication 1, comprenant les étapes de :
(a) préparer, à partir d'une poudre fine d'un ingrédient d'ampoule transmettant la lumière et d'une poudre fine d'un ingrédient de noyau, une suspension d'ingrédient d'ampoule dans laquelle l'ingrédient d'ampoule transmettant la lumière est plus grand que l'ingrédient du noyau, une suspension d'ingrédient du noyau dans laquelle l'ingrédient du noyau est plus grand que l'ingrédient d'ampoule transmettant la lumière, et au moins une suspension intermédiaire dans laquelle l'ingrédient d'ampoule transmettant la lumière et l'ingrédient du noyau ont des proportions compositionnelles se trouvant entre celles de ladite suspension d'ingrédient d'ampoule et de ladite suspension d'ingrédient de noyau ;
(b) former un corps stratifié non cuit composé d'une couche de région côté ampoule non cuite qui doit être disposée adjacente à ladite ampoule transmettant la lumière et formée à partir de ladite fonction d'ingrédient d'ampoule, une couche de région côté noyau non cuite qui doit être disposée adjacente audit noyau et formée à partir de ladite suspension d'ingrédient de noyau, et au moins une couche de région intermédiaire non cuite disposée entre ladite couche de région côté ampoule non cuite et ladite couche de région côté noyau non cuite et formée à partir de ladite au moins une suspension intermédiaire ; et
(c) cuire ledit corps stratifié non cuit ;
(d)
dans lequel ladite étape (b) comprend l'étape de
(g) verser successivement ladite suspension d'ingrédient de noyau, ladite au moins une suspension intermédiaire et ladite suspension d'ingrédient d'ampoule dans un moule qui comprend un corps tubulaire monté verticalement sur une plaque poreuse pour former ladite couche de région côté noyau, ladite couche de région intermédiaire, et ladite couche de région côté ampoule, respectivement, formant de ce fait ledit corps stratifié non cuit.

23. Procédé selon la revendication 22, dans lequel ladite étape (g) comprend l'étape de :
placer verticalement une barre de moule conique au centre dans ledit moule pour définir un trou traversant dans ladite enceinte pour que ledit noyau s'étende à travers celle-ci.

24. Procédé selon la revendication 22, dans lequel ladite étape (c) comprend les étapes de :
mouler une ampoule non cuite à partir de la poudre fine de l'ingrédient d'ampoule transmettant la lumière, et raccorder ledit corps stratifié non cuit à une extrémité ouverte de ladite ampoule non cuite.

25. Procédé selon la revendication 22, dans lequel ladite étape (a) comprend les étapes de :
préparer une suspension d'ampoule pure à partir de la poudre fine du type d'ingrédient d'ampoule transmettant la lumière et former un corps tubulaire d'ampoule non cuit qui doit être formé dans ladite ampoule transmettant la lumière à partir de la suspension d'ampoule pure ;
dans lequel ladite étape (g) comprend l'étape de:
après que ledit corps stratifié non cuit composé de ladite couche de région côté noyau, de ladite couche de région intermédiaire et de ladite couche de région côté ampoule ait été formé, placer solidairement ledit corps d'ampoule non cuit sur ladite couche de région côté ampoule dudit corps stratifié non cuit ; et
dans lequel ladite étape (c) comprend l'étape de :
cuire ledit corps stratifié non cuit incluant ledit corps tubulaire d'ampoule non cuit.
